# EUROPEAN PATENT SPECIFICATION

(11) **EP 0 283 114 B1**
(45) Date of publication and mention of the grant of the patent: **25.08.1993**
(21) Application number: 88300516.7
(22) Date of filing: 22.01.1988
(51) Int. Cl.: D06P 1/673, D06P 3/66

(54) **Alkalizer for fibre reactive dyes in cotton**
Alkalisierungsmittel für faserreaktive Farbstoffe in Baumwolle
Agent d'alcalinisation pour colorants réagissant sur la fibre de coton

(30) Priority: 17.02.1987 US 15428
(43) Date of publication of application: 21.09.1988
(73) Proprietor: SYBRON CHEMICAL HOLDINGS INC., Wilmington, Delaware 19899 (US)
(72) Inventor: De Guzman, Ernesto V., Spartanburg South Carolina 29301 (US); Moran, James C., Taylors South Carolina 29687 (US)
(74) Representative: Ackroyd, Robert

(56) References cited:
- FR-A- 2 148 294
- DATABASE WPIL, no.81-42770D,Derwent Publications Ltd, London, GB

## Description

### Background of the Invention

In the dyeing of cellulosic materials using fibre-reactive dyes, it is the practice to add the cellulosic material and dye to the dyebath first. Next a neutral salt (e.g. sodium sulfate or sodium chloride) is added and the bath is stirred and heated to a prescribed temperature for a prescribed period of time. During this period of time, the dye becomes absorbed by the material as the result of the "salting out" effect of the salt which had been added. This "salting out" step is essential for placing dye molecules in very close proximity to the macromolecules of the cellulosic materials. At this point, the material has absorbed the dye, but the dye is not held fast to the fibre.

After the salt addition and stirring as prescribed, an alkaline material is added to promote a chemical reaction between the dye molecules and atoms of the cellulosic fibres. As a result of this reaction, the dye combines chemically with the cellulosic material. The dye, so bonded, will not wash out of the cellulose. This is known as a "wash-fast" dyeing. Without the "salting out", which increases the substantivity of unreacted dye molecules with the fibre, much of the dye would not have reacted with the fibre and the colour would have been lost.

A fibre-reactive dye molecule is made up of a colour portion and a chemically-reactive portion. When used to dye cellulosic materials, the chemically-reactive portion reacts with an hydroxyl group on the cellulose macromolecule under alkaline conditions to form a chemical bond between the cullulosic material and the colour portion of the dye molecule.

In order to ensure a good yield of dyeing, electrolytes in the form of neutral salts are added to the dyebath to enhance the substantivity of the dye molecules on to the cellulosic material fibres, before chemical reaction between the hydroxyl groups and the chemically-reactive portion of the dye takes place.

Addition of an alkaline material then, under proper conditions of time and temperature, causes the absorbed dye molecules to react with the hydroxyl groups of the cellulosic fibres to form chemical bonds between the dye molecule and the macromolecules of cellulose. There is also a tendency for the dye molecule to react with other hydroxyl groups, such as are present in water. This is known as hydrolysis. When this occurs, the water molecule becomes chemically bonded to the colour portion of the dye molecule, and hence, the dye molecule is lost for combining with the cellulose. The colour washes out of the cellulosic material. Hydrolysis thus results in a lower colour yield on the cellulosic material.

A good yield in dyeing, then, depends on causing a large proportion of the dye molecules to absorb, or "salt out", on to the cellulosic macromolecules, before chemical reaction occurs. This must then be followed by the addition of an alkaline material which promotes the chemical reaction between the cellulosic fibre and the dye molecule and minimizes the reaction between dye molecules and water molecules.

In the past, a number of chemicals have been used as the alkalizing material. For example, sodium hydroxide alone or in combination with soda ash (sodium carbonate); sodium carbonate alone; trisodium phosphate; sodium bicarbonate; tripotassium phosphate alone or in combination with a strong base such as potassium hydroxide and/or sodium hydroxide.

JP-A-56-043490 discloses a resist or discharge printing paste containing, as indispensable ingredients, an alkali metal salt, fine silica powder and an alkaline compound which is preferably sodium or potassium carbonate or hydroxide or sodium or potassium phosphate.

FR-A-2148294 states that known acid binding agents used in dyeing with reactive dyestuffs are caustic alkalis, sodium carbonate, sodium bicarbonate, trisodium phosphate and sodium metasilicate.

### Summary of the Invention

The present invention provides an alkalizer, suitable for use as a textile bath additive which comprises a water solution containing tripotassium phosphate, characterised in that the alkalizer comprises a premixed liquid composition suitable for direct addition to a textile bath and being formed from, by weight:

| | |
|---|---|
| Tripotassium phosphate | 5-45% |
| Potassium hydroxide and/or sodium hydroxide | 0-10% |
| Potassium carbonate and/or sodium carbonate | 2-10% |
| Water | Balance |

This invention also provides a method of controlling the alkali content of a reactive dye bath process, which comprises:
(a) providing a liquid reactive dye-bath solution which contains water, surfactant, salt and a dye,
(b) placing in the bath a cellulose-containing textile material to be dyed and heating the dye-bath for a prescribed period of time, and
(c) adding an alkalizer to the bath, characterised in that the alkalizer comprises a premixed liquid solution which is formed from, by weight, from 5 to 45% of tripotassium phosphate, up to 10% of potassium hydroxide and/or sodium hydroxide, and from 2 to 10% of potassium carbonate and/or sodium carbonate, with the balance water, the alkalizer being present in an amount sufficient to control the alkali concentration of the dye-bath at a level sufficient to allow the reactive dye to form a firm chemical bond with the cellulose-containing textile material when heated for a prescribed period of time.

It has thus been discovered that a combination of tripotassium phosphate (K₃PO₄), optionally potassium hydroxide (KOH) and/or sodium hydroxide (NaOH), plus potassium carbonate (K₂CO₃) and/or sodium carbonate (Na₂CO₃), when used in the specified amounts as an alkalizer for dyeing cellulosic material with fibre-reactive dyes, yields dyeings with less hydrolysis and therefore increased yield of colour on the cellulose.

It has been further discovered that the combination of these ingredients can be made as a convenient direct textile bath additive in the form of an aqueous solution, preferably with a total solids ranging from about 10% up to approximately 50% by weight of the solution. The limit of lower percentage is dictated by the economics of having a more concentrated solution for transportation. The upper limit of concentration is determined by the temperature at which a mixture can be stored. For storage above 10°C, the concentration can be even higher.

### Detailed Description of the Invention

The liquid alkalizer of the present invention can be formulated over a wide range of concentrations. It has been found that the combination of the ingredients of the present invention can be made in aqueous solutions, preferably with the total solids ranging from about 10% to up to approximately 50% by weight of the solution. The lower limit is dictated mainly by the economics of having a more concentrated solution for transportation, while the upper limit of concentration is determined by the temperature at which a mixture can be stored. For storage above 10°C, the concentration can be higher. It has been found that a combination of K₃PO₄, KOH and/or NaOH plus K₂CO₃ and/or Na₂CO₃ , when used in combination as an alkalizer for dyeing a cellulosic material with fibre-reactive dyes, provides dyeings with less hydrolysis and therefore increased yield of colour on the cellulose.

The broad and preferred concentration ranges for the K₃PO₄, KOH and/or NaOH and K₂CO₃ and/or Na₂CO₃ for liquid alkalizers of the present invention are tabulated below in weight percent of the solution:

| | Broad Range | Preferred Range |
|---|---|---|
| K₃PO₄ | 5-45% | 10-35% |
| KOH and/or NaOH | 0-10% | 2-8% |
| K₂CO₃ and/or Na₂CO₃ | 2-10% | 3-8% |
| Water: | Balance | Balance |

Although the potassium hyroxide (or equivalent sodium hydroxide) is optional, it is a preferred component in that it functions in the dye-bath to neutralize acidity.

NaOH may be fully or partially substituted to an equal total amount for KOH and Na₂CO₃ may be fully or partially substituted to an equal total amount for the K₂CO₃.

A typical method used for making the liquid alkalizers of the present invention is as follows: To prepare a formulation of the present invention, the appropriate amount of water is first added to a vessel. The K₃PO₄ can be added with stirring and, when dissolved, the desired amount of KOH is then added. Next, Na₂CO₃ or K₂CO₃ is added. The alkalizer mix is stirred and drained into drums after cooling below 40°C. The drummed material is the alkalizer ready for use or sale.

As an alternative to adding solids, the liquid alkalizer can be prepared using phosphoric acid (H₃PO₄), a 45% solution of KOH and a 47% solution of K₂CO₃, all of which are commercially available.

The water content of the alkalizer of the present invention can therefore originate from water introduced as such, or from water introduced as part of an aqueous solution of the other ingredients, or partly from one source and partly from the other.

For example, formula (A) of TABLE II would be made as follows:

The ingredients would be added in the same order as listed, using cooling as necessary to keep temperature below 70°C. Cool to 40°C and pack into drums.

Formula (F) of TABLE II would be made as follows:
8.1% Water
61.8% KOH - 45% solution
21.6% H₃PO₄ - 75% solution
8.5% K₂CO₃ 47% solution
Add ingredients in the order listed, using cooling to keep the temperature below 70°C. Cool finally to below 40°C and pack into drums.

The alkalizer formulations of the present invention may be used for the dyeing of cellulosic materials with fibre-reactive dyes as follows, using an Ahiba Laboratory dyeing apparatus to carry out the dyeing:
Into a suitable dyeing beaker of about 230 ml volume, 100 ml of water at 80°F (27°C), 7 grams of sodium chloride, 0.05 grams of surfactant, Tanaterge LV (Sybron Chemicals, Inc), and 0.3 grams of Remazol REd F3B Fibre-Reactive Dye (American Hoechst) are added. Place the beaker in the water bath of the Ahiba device. Mount a swatch of 100% woven cotton on an agitator holder and insert it into the beaker. The agitator is capable of simultaneous vertical and rotational motion. The cotton swatch in held below the surface of the liquid at the lowest point of the agitator movement. The Ahiba bath is held at 80°F (27°C) while agitating for 10 minutes. Then about 0.5 gm of liquid alkalizer is added and the bath is agitated for 10 minutes. The bath is then heated to 140°F (60°C), and agitated for 45 minutes. The cotton swatch is then removed from the bath, washed with cold water, then hot water, then soap solution, then hot water and finally cold water. The swatch is then dried and the dyed colour evaluated.

The above dyeing technique is used with three different alkalizers. These three alkalizers are formulas (A), (B), and (G) of TABLE II. Formula (G) is a Sybron Chemicals, Inc. commercial alkalzier sold under the trademark ALKAFLO®. Using the ALKAFLO alkalizer as the reference standard alkalizer, the colours of 100% cotton swatches are compared and tested by means of the ACS Spectro Sensor (Applied Color Systems Inc.).

A specific description of the evaluation of the comparative test data obtained from the results is set forth in TABLE I.

The dry dyed cotton sample was folded over twice and then placed in the sample holder of the ACS Spectro Sensor. A scan of the sample is then run automatically and the spectro data automatically stored in the IBM PC computer which is connected to the ACS Sensor.

The cotton sample which was dyed using ALKAFLO liquid alkalizer as the alkalizer is arbitrarily taken as the standard, with the strength reading set at 100. The spectro data of the other samples are compared automatically by the IBM PC and strength results are printed out.

Readings of 100 are equal to standard. Readings above 100 show greater dye strength than standard. Readings below 100 show weaker dye strength than standard.

The results of dyeing using Remazol Red F3B with three different alkalizers are listed below in the TABLE I:

**TABLE I**

| ALKALIZER | STRENGTH |
|---|---|
| Formula G | 100 |
| Formula A | 105 |
| Formula B | 101 |

It can be seen from the above TABLE I that the formulas of the present invention result in greater dye strength than the standard.

The following formulations (A) to (F) in TABLE II below represent typical examples of suitable liquid alkalizer compositions of the present invention in weight percent:

A small amount, such as 0.1%, of sodium gluconate or other suitable sequestering agent may be added to any of the above formulations, to prevent the formation of precipitates caused by impurities in the water or chemicals used.

## Claims

1. An alkalizer, suitable for use as a textile bath additive which comprises a water solution containing tripotassium phosphate, characterised in that the alkalizer comprises a premixed liquid composition suitable for direct addition to a textile bath and being formed from, by weight:
| | |
|---|---|
| Tripotassium phosphate | 5-45% |
| Potassium hydroxide and/or sodium hydroxide | 0-10% |
| Potassium carbonate and/or sodium carbonate | 2-10% |
| Water | Balance |

2. An alkalizer composition according to claim 1, which is formed from tripotassium phosphate, potassium hydroxide, potassium carbonate and water.

3. An alkalizer composition according to claim 1, which is formed from tripotassium phosphate, sodium hydroxide and sodium carbonate and water.

4. An alkalizer composition according to any preceding claim, which is formed from water and, by weight:
| | |
|---|---|
| Tripotassium phosphate | 10-35% |
| Potassium hydroxide and/or sodium hydroxide | 2-8% |
| Potassium carbonate and/or sodium carbonate | 3-8% |

5. An alkalizer composition according to any preceding claim, having a total solids content of from 10 to 50% by weight.

6. A method of controlling the alkali content of a reactive dye bath process, which comprises:
(a) providing a liquid reactive dye-bath solution which contains water, surfactant, salt and a dye,
(b) placing in the bath a cellulose-containing textile material to be dyed and heating the dye-bath for a prescribed period of time, and
(c) adding an alkalizer to the bath, characterised in that the alkalizer comprises a premixed liquid solution which is formed from, by weight, from 5 to 45% of tripotassium phosphate, up to 10% of potassium hydroxide and/or sodium hydroxide, and from 2 to 10% of potassium carbonate and/or sodium carbonate, with the balance water, the alkalizer being present in an amount sufficient to control the alkali concentration of the dye-bath at a level sufficient to allow the reactive dye to form a firm chemical bond with the cellulose-containing textile material when heated for a prescribed period of time.

7. A method according to claim 6, in which the alkalizer is formed from tripotassium phosphate, potassium hydroxide and potassium carbonate and water.

8. Method according to claim 6, in which the alkalizer is formed from tripotassium phosphate, sodium hydroxide and sodium carbonate and water.

9. A method according to any of claims 6 to 8, in which the alkalizer is formed from water and, by weight:
| | |
|---|---|
| Tripotassium phosphate | 10-35% |
| Potassium hydroxide and/or sodium hydroxide | 2-8% |
| Potassium carbonate and/or sodium carbonate | 3-8% |

10. A method according to any of claims 6 to 9, in which the alkalizer has a total solids content of from 10 to 50% by weight at the time of its addition to the bath.

## Patentansprüche

1. Als Textilbadadditiv geeignetes Alkalisierungsmittel, welches aus einer, Trikaliumphosphat enthaltenden wässrigen Lösung besteht, dadurch gekennzeichnet, daß das Alkalisierungsmittel aus einer zum direkten Einbringen in ein Textilbad geeigneten, aus
- 5 Gew.-% bis 45 Gew.-% Trikaliumphosphat
0 Gew.-% bis 10 Gew.-% Kaliumhydroxyd und/oder Natriumhydroxyd
2 Gew.-% bis 10 Gew.-% Kaliumkarbonat und/oder Natriumkarbonat
und im übrigen aus Wasser hergestellten, vorgemischten flüssigen Zusammensetzung besteht.

2. Alkalisierungszusammensetzung nach Anspruch 1, hergestellt aus Trikaliumphosphat, Kaliumhydroxyd, Kaliumkarbonat und Wasser.

3. Alkalisierungszusammensetzung nach Anspruch 1, hergestellt aus Trikaliumphosphat, Natriumhydroxyd, Natriumkarbonat und Wasser.

4. Alkalisierungszusammensetzung nach einem der vorangegangenen Ansprüche, hergestellt aus Wasser und
- 10 Gew.-% bis 35 Gew.-% Trikaliumphosphat,
2 Gew.-% bis 8 Gew.-% Kaliumhydroxyd und/oder Natriumhydroyd und
3 Gew.-% bis 8 Gew.-% Kaliumkarbonat und/oder Natriumkarbonat.

5. Alkalisierungszusammensetzung nach einem der vorangegangenen Ansprüche mit einem Gesamtgehalt an Feststoffen von 10 Gew.-% bis 50 Gew.-%.

6. Verfahren zur Regelung des Alkaligehalts eines reaktiven Färbebadprozesses, bestehend aus
(a) der Bereitstellung einer flüssigen reaktiven Färbebadlösung, welche Wasser, ein oberflächenaktives Mittel, Salz und einen Farbstoff enthält,
(b) dem Einbringen eines zellulosehaltigen textilen, zu färbenden Materials in das Bad sowie der Aufheizung des Färbebades während einer vorgeschriebenen Zeitspanne und
(c) dem Einbringen eines Alkalisierungsmittels in das Bad, dadurch gekennzeichnet, daß das Alkalisierungsmittel eine vorgemischte flüssige Lösung umfaßt, die aus 5 Gew.-% bis 45 Gew.-% Trikaliumphosphat, bis zu 10 Gew.-% Kaliumhydroxyd und/oder Natriumhydroxyd und aus 2 Gew.-% bis 10 Gew.-% Kaliumkarbonat und/oder Natriumkarbonat hergestellt ist, wobei der Rest Wasser ist, wobei das Alkalisierungsmittel in einer solchen Menge eingesetzt wird, welche zur Regelung der Alkalikonzentration des Färbebades auf einem solchen Niveau ausreichend ist, welches die Bildung einer festen chemischen Verbindung des reaktiven Farbstoffes mit dem zellulosehaltigen textilen Material ermöglicht, sobald das Bad während einer vorgeschriebenen Zeitspanne beheizt wird.

7. Verfahren nach Anspruch 6, bei welchem das Alkalisierungsmittel aus Trikaliumphosphat, Kaliumhydroxyd, Kaliumkarbonat und Wasser gebildet ist.

8. Verfahren nach Anspruch 6, bei welchem das Alkalisierungsmittel aus Trikaliumphosphat, Natriumhydroxyd, Natriumkarbonat und Wasser gebildet ist.

9. Verfahren nach einem der Ansprüche 6 bis 8, bei welchem das Alkalisierungsmittel aus Wasser und
- 10 Gew.-% bis 35 Gew.-% Trikaliumphosphat,
2 Gew.-% bis 8 Gew.-% Kaliumhydroxyd und/oder Natriumhydroxyd und
3 Gew.-% bis 8 Gew.-% Kaliumkarbonat und/oder Natriumkarbonat
hergestellt ist.

10. Verfahren nach einem der Ansprüche 6 bis 9, bei welchem das Alkalisierungsmittel zur Zeit des Einbringens in das Bad einen gesamten Feststoffgehalt von 10 Gew.-% bis 50 Gew.-% aufweist.

## Revendications

1. Agent d'alcalinisation, convenant pour l'utilisation comme additif de bain pour textiles qui comprend une solution aqueuse contenant du phosphate tripotassique, caractérisé en ce que l'agent d'alcalinisation comprend une composition liquide prémélangée convenant pour l'addition directe à un bain pour textiles et étant formée de, en poids
| | |
|---|---|
| phosphate tripotassique | 5-45% |
| hydroxyde de potassium et/ou hydroxyde de sodium | 0-10% |
| carbonate de potassium et/ou carbonate de sodium | 2-10% |
| eau | complément |

2. Composition d'agent d'alcalinisation selon la revendication 1, qui est formée de phosphate tripotassique, d'hydroxyde de potassium, de carbonate de potassium et d'eau.

3. Composition d'agent d'alcalinisation selon la revendication 1, qui est formée de phosphate tripotassique, d'hydroxyde de sodium et de carbonate de sodium et d'eau.

4. Composition d'agent d'alcalinisation selon l'une quelconque des revendications précédentes, qui est formée d'eau et de, en poids,
| | |
|---|---|
| phosphate tripotassique | 10-35% |
| hydroxyde de potassium et/ou hydroxyde de sodium | 2-8% |
| carbonate de potassium et/ou carbonate de sodium | 3-8% |

5. Composition d'agent d'alcalinisation selon l'une quelconque des revendications précédentes, ayant une teneur totale en matières solides de 10 à 50% en poids.

6. Procédé de maîtrise de la teneur en matières alcalines dans un traitement par un bain de colorant réactif, qui consiste,
a) à fournir une solution de bain de colorant réactif liquide qui contient de l'eau, du surfactif, du sel et un colorant,
b) à placer dans le bain un matériau textile contenant de la cellulose à teindre et à chauffer le bain de teinture pendant une période de temps prescrite, et
c) à ajouter au bain un agent d'alcalinisation,
caractérisé en ce que l'agent d'alcalinisation comprend une solution liquide prémelangée qui est formée de, en poids, 5 à 45% de phosphate tripotassique, jusqu'à 10% d'hydroxyde de potassium et/ou d'hydroxyde de sodium, et 2 à 10% de carbonate de potassium et/ou de carbonate de sodium, le complément étant de l'eau, l'agent d'alcalinisation étant présent en quantité suffisante pour maîtriser la concentration en matières alcalines du bain de teinture à un niveau suffisant pour permettre au colorant réactif de former une liaison chimique ferme avec le matériau textile contenant de la cellulose quand il est chauffé pendant une période de temps prescrite.

7. Procédé selon la revendication 6, dans lequel l'agent d'alcalinisation est formé de phosphate tripotassique, d'hydroxyde de potassium et de carbonate de potassium et d'eau.

8. Procédé selon la revendication 6, dans lequel l'agent d'alcalinisation est formé de phosphate tripotassique, d'hydroxyde de sodium et de carbonate de sodium et d'eau.

9. Procédé selon l'une quelconque des revendications 6 à 8, dans lequel l'agent d'alcalinisation est formé d'eau et de, en poids,
| | |
|---|---|
| phosphate tripotassique | 10-35% |
| hydroxyde de potassium et/ou hydroxyde de sodium | 2-8% |
| carbonate de potassium et/ou carbonate de sodium | 3-8% |

10. Procédé selon l'une quelconque des revendications 6 à 9, dans lequel l'agent d'alcalinisation a une teneur totale en matières solides de 10 à 50% en poids, au moment de son addition au bain.
